

Sept. 1, 1925.

1,551,966

**P. C. MULLIGAN ET AL.**  
PROCESS OF PREPARING MATERIALS FOR BRIQUETTING  
AND THE PRODUCT THEREOF  
Filed Nov. 14, 1923



## Inventors

Paul C. Mulligan  
Herbert E. Swalwell  
By H. L. & C. L. Reynolds  
Attorne

Attorneys

## UNITED STATES PATENT OFFICE.

PAUL C. MULLIGAN AND HERBERT G. SWALWELL, OF SEATTLE, WASHINGTON, AS-SIGNORS TO THEMSELVES, LUTHER J. HULL, AND ISAAC M. FOSTER, ALL OF SEATTLE, WASHINGTON.

## PROCESS OF PREPARING MATERIALS FOR BRIQUETTING AND THE PRODUCT THEREOF.

Application filed November 14, 1923. Serial No. 674,704.

*To all whom it may concern:*

Be it known that we, PAUL C. MULLIGAN and HERBERT G. SWALWELL, citizens of the United States of America, and residents of the city of Seattle, in the county of King and State of Washington, have invented certain new and useful Improvements in Processes of Preparing Materials for Briquetting and the Product Thereof, of which the following is a specification.

Our invention relates to the art of briquetting, and particularly to the preparation of materials for briquetting.

Our invention is more especially designed for the utilization of waste products such as saw dust or wood chips, and will be described with particular relation thereto. However, in the following specification and in the claims terminating the same, it will be understood that the term "granular material" is intended to apply either to saw dust or to wood chips in the natural state, or dried or charred, and either separated or in combination, or to other combustible matter in a divided form, which it is desired to finally compress into the form of a briquet.

One of our principal objects is the provision of a process whereby such granular materials may be prepared for briquetting through the use of a solid binder which may be supplied in a pulverized form and without heating, rather than in a liquid form, as has been customary heretofore, rendering it possible to employ an air current for handling this pulverized binder, and making it possible also to employ a simple beater type of pulverizer for the pulverization of such solid binder without danger of fouling the screens employed in such a pulverizer.

A further object is the provision of a process for the preparation of materials for briquetting, whereby the fuel value and the amount of flame-producing volatiles in the final briquet may be increased by the addition thereto of a liquid hydrocarbon, as fuel oil, in such a manner that it will remain in the briquet and will not exude therefrom or render the briquet moist or sticky.

A further object is the provision of a process for preparing materials for briquetting, which may be carried on continuously, without interruption, to the end that the

materials prepared for compressing or briquetting may be continuously fed to a continuously acting briquetting press.

A further object is the provision of a novel mixture of materials intended for briquetting.

A further object is the provision of a novel article of manufacture consisting of a briquet having a novel combination of ingredients therein.

While our process is designed to supply materials to a briquetting press such as is disclosed in our application for patent upon the same, Serial No. 674,705 filed coincidentally with the present application, yet it will be understood that the use of this particular piece of apparatus is not essential to the process, nor in fact, is it essential that any particular form of apparatus be employed in carrying out the same. The apparatus which we have illustrated diagrammatically in the accompanying drawings represents only a form which might conveniently be employed in carrying out the process.

Our invention comprises the novel steps, combinations and arrangements thereof in the process of preparing materials for briquetting, and in the novel mixture for briquetting and the novel briquet formed from such mixture, all as disclosed in this specification and in the claims terminating the same.

Figure 1 represents diagrammatically a complete plant for the carrying out of our process of briquetting.

Figure 2 represents a transverse section through a beater type of pulverizer, illustrating a form which may conveniently be employed in carrying out our process, although it will be understood that the use of this particular type of apparatus is not essential.

As we have stated above the base material which is in granular form, will preferably be carbonized wood saw-dust or chips. The saw-dust is generally considered a waste product and it is to utilize this waste that our process is particularly intended. It should be understood, however, that we do not consider that our process is limited only to the utilization of such materials, and in fact, we have found it adaptable to the briquetting of such materials as ordinary

- ground charcoal or coal. Also we may wish to utilize other combustible materials which are ordinarily wasted, and for that reason have chosen the term "granular material", 5 as representing a material or several materials in granular form, generally of vegetable origin, and combustible, which it is desired to incorporate into a briquet as the base thereof.
- 10 The material, if saw-dust or chips or like material is used, is first dried. We have shown in the drawings no means of drying the granular material, nor in fact, do we consider this strictly a part of our process, 15 but merely a preliminary step which must be taken if the material requires it. Preferably the material is dried to the point of charring. After drying the material may be stored in a convenient place, as in a storage bin 1, from which it is fed as required into the hopper 20 of a mixing chamber 2. As it enters the chamber 2 a liquid hydrocarbon, as, for example, fuel oil, may be supplied thereto. The oil is supplied for the 20 purpose of adding volatile matter to the briquet, and its use for some briquets may be dispensed with, although preferably it is employed.
- The oil we have shown as being supplied 30 from a tank 3 by means of a conduit 30, and we have shown a conduit 40 for air which is contained in a holder 4 under pressure, which also communicates at 31 to a spray nozzle with which the oil conduit 30 is connected. By this means the oil, the supply 35 of which may be controlled, as by a valve 32, is sprayed into and upon the granular material as it enters the mixing chamber 2. The oil and dry granular material are suitably 40 mixed, as by a screw 21 within the chamber 2, and finally when the mixing has progressed sufficiently that the oil impregnates the dry granular material, the oil-moistened granular material is delivered to a second 45 mixing chamber 5.
- During the time that the oil and granular material are being mixed, a binder therefor, which preferably consists simply of normally solid asphalt, is being prepared for 50 mixture therewith. In the drawings 60 represents the casing of a common beater type pulverizer. In such a pulverizer, beaters 6 of hard metal are pivoted upon the ends of arms 61, which in turn are pivoted upon a rotatable hub 62. Material to be pulverized is fed into a hopper 63 at the top of the casing 60 and as the beaters 6 rotate close to the interior of the casing 60, the solid materials are pulverized and finally dropped 55 through a screen 64 forming the bottom of the casing 60. There they are received in a chamber 65 from which they are drawn generally by the suction of a blower 66 and are then delivered to a conduit 67.
- 60 The conduit 67 connects either directly or through a separator 68 with the chamber 5. The pulverized asphalt enters the chamber 5 at substantially the same point as the oil-moistened granular material, and preferably is carried thence by an air current from the 70 blower 66. The pulverized material is deposited upon the moist granular material and the air which serves as a vehicle therefore passes through the chamber 5, which should be closed, and during its passage the 75 air is relieved of all of the pulverized material. It is permitted to escape through a screened opening 50.
- Within the chamber 5 the pulverized 80 binder and the granular base are thoroughly mixed to disseminate the binder throughout the mixture. This may be done by means of a second screw conveyor 51 within the chamber 5. The material is then ready for briquetting and may be delivered from the 85 chamber 5 continuously into a hopper 73 of a briquetting press, indicated in general by the numeral 7, which, operating continuously, will produce briquets from the material thus prepared. For convenience we 90 have shown the briquetting press 7 as containing a cylinder 70 in which, by means of a piston, not shown, it is possible to compress air to be delivered through a conduit 95 74 to the air storage tank 4.
- It has heretofore been considered impossible to use asphalt as a binder for briquetting in the solid form, and without heating. This has been for the reason that the asphalt 100 has always tended to clog the screens of pulverizers employed to reduce it to a powdered form. We have discovered, however, that by means of the addition to the pulverizer 60 of a more friable material as, for instance, charcoal or coal, in about the same or slightly greater amounts by weight than the asphalt, but perhaps twice the bulk thereof, it is possible to pulverize the asphalt and the friable material in conjunction with each other, and thereby to render the particles of asphalt so much less sticky than they normally would be that there will be no tendency to clog the screens, as 64. The action 105 appears to be that the friable material, being most readily broken up, has a portion pulverized first, before any pulverization of the asphalt begins. The particles of the friable material, then act to coat the asphalt and to coat the particles thereof as formed in such manner that the stickiness of the asphalt is removed, or the asphalt particles are enclosed within a casing of fine particles of the friable material and thus do not cohere into a mass nor adhere to the screen surface. 110 This renders it possible to use this simple and convenient type of pulverizer as described and renders it possible also to convey the pulverized material by means of an air current to the desired point where it is mixed with the granular base. It removes 115 120 125 130

any tendency for the asphalt to stick in any part of the apparatus employed.

A number of different materials may be used to prevent stickiness of the asphalt binder. We have mentioned coal and charcoal as being suitable for such use, and prefer to use them for the reason that these materials are combustible as is the asphalt, thus rendering the entire briquet combustible. It should be understood, however, that we do not limit ourselves strictly to the use of these two materials as a vehicle or separator for the asphalt particles, but prefer them on account of their combustibility. When other materials are thus employed, the amount employed is determined chiefly by their bulk, sufficient friable material being used to properly coat and separate the binder and its particles in the manner described above.

As a substitute for asphalt we have used other solid binder materials, for example, pitch, both coal tar pitch and resins. We do not wish to be limited, therefore, solely to the use of asphalt as a binder. When pitch is employed, it is still desirable to employ charcoal or the like as a separating medium for the individual particles of the binder material, and to pulverize the charcoal and binder materials together. The charcoal, in this capacity, acts to separate the individual binder particles, to permit handling and to prevent reaccumulation thereof.

In brief, then, the complete process consists of the impregnation of the granular base with a liquid hydrocarbon, coincidentally with which impregnation there is a pulverization of the asphalt and of charcoal to form a combustible carbon carrier or separator therefor, following which the pulverized materials and the oil-moistened granular materials are mixed thoroughly. The final mixture is then ready to be supplied to a suitable press and upon compression a briquet is formed, which is dry, not sticky, which is fairly hard, and which will not break down while burning.

In compressing the briquetting mixture which we have described, the increased density caused by compression appears to be sufficient to bring the particles of the sticky asphalt binder closely enough together to cause cohesion of all the granular particles, and as well, of the pulverized carbon which has been put into the mixture with the pulverized asphalt.

It is difficult to express the proportions of the ingredients in such a mixture and in the briquet formed therefrom, with any exactness, for the reason that these percentages will vary considerably under varying conditions. For example, the amount of fuel oil will be determined principally by the absorption of the granular base and this in turn will vary with the character of the

granular material, whether coal, charcoal or wood, and with the dryness thereof. Generally speaking, we may employ from 2% to 30% of fuel oil or its equivalent, although generally in the neighborhood of 16% or 17% is most desirable. Of the asphalt binder, the amount will vary with the pressure employed in the briquetting press, and also it will depend to some extent on the amount of fuel oil employed, a greater amount of fuel oil tending to keep the granules of the base material separate and requiring a slightly greater amount of binder. Generally speaking, from 7% to 15% of the asphalt binder will be employed under different conditions, with the preferred amount about 11%, when using carbonized saw-dust and fuel oil as the other constituents. The remainder (with the exception of the amount of carbon which is added with the pulverized asphalt, the percentage of this being substantially the same as of asphalt) will be the granular base. This, as stated above, might be charcoal or coal or such material in combination with sawdust or wood chips. Granular charcoal, including that introduced into the mixture with the asphalt, may be employed in an amount necessary to complete the mixture, and preferably should be present in an amount approximately 73% of the weight of the briquet. If other materials are substituted for a part of the charcoal, the percentage of the latter is reduced accordingly. The percentages given are all by weight.

What we claim as our invention is:

1. A process of preparing fuels for briquetting which consists in pulverizing a combustible solid binder material, at the same time impregnating a granular combustible base with a liquid hydrocarbon, introducing the pulverized binder immediately to the moistened base, and finally mixing them to disseminate the binder throughout the mixture.

2. A continuous process of preparing fuels for briquetting which consists in pulverizing an asphalt binder in conjunction with carbon, at the same time impregnating charcoal with fuel oil, introducing the pulverized materials by an air current to the oiled charcoal, whereby the pulverized material is deposited, and then mixing the pulverized material and charcoal to disseminate the former throughout the mixture.

3. A continuous process for the formation of a fuel briquet which consists in pulverizing a combustible binder in the cold state, in mixing a granular base material with said pulverized binder to disseminate the binder throughout the mixture, and finally compressing it while cold to cause adhesion of the particles.

4. The process of preparing fuels for briquetting with a normally solid binder mate-

rial which consists in pulverizing the binder material in conjunction with carbon, in delivering the pulverized materials to a granular base by means of an air current, the granular base having been moistened by oil just prior, whereby the pulverized material is arrested, and in then mixing the pulverized and granular material.

5. A briquetting process which consists in 10 pulverizing a normally solid binder while cold and in its normal solid state, together with a more friable material, mixing the pulverized materials with a briquet base, and compressing the mixture while cold to cause 15 the particles to cohere.

6. A briquetting mixture comprising a granular combustible base impregnated with oil, and a combustible binder in pulverized form thoroughly mixed therewith.

20 7. A briquetting mixture comprising a granular combustible base impregnated with a liquid hydrocarbon, and a pulverized combustible binder commingled with a pulverized combustible vehicle therefor, and thoroughly mixed with the base.

25 8. A briquet comprising fuel oil, an asphalt binder, a quantity of pulverized carbon, and the remainder charred wood sawdust or chips, the amount of oil being limited 30 by the absorption of the charred wood, the

quantity of carbon being sufficient to retain the asphalt in a pulverized condition until compressed, and the quantity of binder being sufficient to cause cohesion of the charred wood particles when the mixture is compressed.

35 9. A briquet comprising fuel oil from 2% to 30% by weight, between 7% and 15% of asphalt binder, and the remainder a combustible base in finely divided form, the 40 amount of fuel oil being in any preferred proportion up to the limit of absorption thereof by the base, and the percentage of binder being sufficient to cause the oil impregnated particles of the base to cohere 45 when compressed.

10. A briquet including fuel oil approximately 16% or 17% by weight, about 11% of asphalt binder, and the remainder a granular combustible base.

50 11. A briquet containing the ingredients in substantially the percentages by weight named, as follows: fuel oil, 16%, asphalt binder, 11%, and carbon 73% in granular and pulverized form.

55 Signed at Seattle, King County, Washington, this 2nd day of November 1928.

PAUL C. MULLIGAN.  
HERBERT G. SWALWELL.